

April 3, 1945.

L. B. LINDEMUTH

2,373,036

METHOD OF CASTING INGOTS

Filed June 30, 1943

*Fig. 1.*



*Fig. 2.*



INVENTOR.  
LEWIS B. LINDEMUTH.

BY  
Benj. T. Rauber  
ATTORNEY.

## UNITED STATES PATENT OFFICE

2,373,036

## METHOD OF CASTING INGOTS

Lewis B. Lindemuth, Port Washington, N. Y.,  
 assignor, by mesne assignments, to Steel Ingot  
 Production, Inc., a corporation of Delaware

Application June 30, 1943, Serial No. 492,953

3 Claims. (Cl. 22—200)

My invention relates to ingot molds and a method of casting ingots of ferrous metals, such as steel or other metals.

Ingots of steel or other ferrous metals are generally cast in iron or steel molds, which may have either an integral or removable bottom. In either case the molten metal upon pouring or teeming into the empty mold strikes the bottom of the mold with considerable force and being at the melting temperature tends to wear away or erode that portion of the bottom of the mold on which it impinges. This has a tendency to form cavities in the mold, or the bottom of the mold, and after cavities have thus been formed or eroded in the mold the cast metal may solidify therein and may partly weld thereto and thus make it difficult to remove the cooled ingot from the mold.

My present invention provides an ingot mold and a method of casting the ingot in such a way as to prevent or minimize this erosion of the bottom surface of the mold and to avoid the tendency of ingots to stick to the mold.

In my invention I protect the bottom surface of the mold cavity with a layer or film of lead in such a manner that when the molten steel, or other ferrous metal, is poured or teemed into the mold it does not strike the metal of the mold directly but instead impinges on the lead.

Inasmuch as the lead melts at a much lower temperature than steel and has a greater density or specific gravity and does not alloy with the steel, it not only protects the bottom of the mold from erosion but when the mold is filled remains as a liquid layer or film between the bottom of the mold and the ingot and does not in any way interfere with the composition of the ingot.

Inasmuch as the lead is liquid it is displaced only temporarily by the molten steel as the latter is poured into the mold and though it may be displaced temporarily by the stream of molten metal it immediately sinks to the bottom of the mold as the filling of the mold proceeds and as the lower part of the metal becomes quiescent. There is, therefore, no erosion effect so far as the lead is concerned.

Owing to its inertia it provides an effective cushion between the poured metal and the inner surface at the bottom of the mold. After the mold and ingot have cooled the ingot may be removed leaving the lead in the mold either as a solidified layer or in the molten condition, depending upon the temperature at which the ingot is removed.

In the case of a mold having a solid or closed bottom, in which case the walls taper downwardly, it is only necessary to put into the mold a sufficient amount of lead to form a layer of the desired depth.

In the case of an open bottom mold closed by a bottom plate or plug, I prefer to provide a lead seal outside of the lower part of the mold through which lead may be displaced by the weight of the molten steel. However, it will be apparent that any other type of bottom closure may be employed.

The various features of my invention are illustrated diagrammatically, by way of example, in the accompanying drawing in which

Fig. 1 is a vertical section of a closed bottom ingot mold embodying my invention, and

Fig. 2 is a similar section of an open bottom mold.

20 Referring to the embodiment shown in Fig. 1 the invention is illustrated as applied to an ingot mold having a bottom 10 and an upstanding or upright wall 11 which tapers downwardly so that the solidified ingot may readily be removed therefrom. The upper end of the mold may be provided with a hot top ring 12. Into the mold there is placed a quantity of metallic lead which melts and forms a pool 13 when the mold is heated above the melting temperature of the lead. It will be understood that if the lead is in a solid or unmelted phase when the teeming is started it may be immediately melted by contact with the highly heated molten steel or other ferrous metal so that it will then form a molten pool at the bottom of the mold. By interposing this pool between the steel being poured and the bottom of the mold the teeming steel must displace or erode the lead before it can reach the bottom of the mold and with a sufficient thickness of lead, depending upon the dimensions of the mold and the conditions of teeming, the force of the poured metal may be expended in displacing the lead without actually contacting with the bottom of the mold or contacting it with such a weak force that no substantial erosion results.

In Fig. 2 the invention is illustrated as applied to an open bottom mold having a vertical wall 14 which tapers upwardly so that the mold can be lifted upwardly from the solidified ingot. The bottom of the mold or mold cavity is closed by a bottom plate 15 spanning the area of the mold and extending below the lower edge of the mold wall and thence upwardly as at 16 to form a narrow channel or moat 17. A layer 18 of molten

lead within the mold 14 may flow or seep into the channel 17 without being lost. When molten steel is poured into the ingot its force or impact will be taken up primarily by the layer of lead 18 and when the latter is entirely molten it might 5 be displaced to a greater or less extent beneath the wall of the ingot 14 and into the moat or channel 17 before the lower part of the molten metal solidifies in the mold. In any event, however, the layer of lead takes the impact of the molten steel and thus protects the bottom plate 15 from erosion. Erosion of the lead is of no consequence because it immediately takes the form of a liquid which does not alloy with or 10 stick to the steel ingot.

Through the above invention the surface of the mold on which the molten metal impinges is protected by a displaceable layer of metal which, having a melting point below that of the steel, assumes a liquid form against which erosion has 15 not permanent effect.

Inasmuch as the lead forms a smooth layer below the cast ingot and does not alloy with it, the ingot may readily be lifted from the bottom wall of the mold.

5 What I claim is:

1. A method of casting ingots of ferrous metal which comprises covering the bottom of an ingot mold cavity with lead and pouring molten ferrous metal into said mold so that the stream of molten ferrous metal impinges directly on the lead.

2. A method of casting ingots of ferrous metal which comprises covering the bottom of an ingot mold cavity with a layer of molten lead and pouring molten ferrous metal into said mold so that the stream of molten ferrous metal impinges directly on the lead.

3. A method of casting ingots of ferrous metal which comprises placing lead in an empty ingot mold and pouring molten ferrous metal into said mold so that the stream of molten ferrous metal impinges directly on the lead.

LEWIS B. LINDEMUTH.